

## UNITED STATES PATENT OFFICE.

KARL P. McELROY, OF WASHINGTON, DISTRICT OF COLUMBIA, ASSIGNOR OF ONE-HALF TO ALFRED M. HOUGHTON, OF WASHINGTON, DISTRICT OF COLUMBIA, AND ONE-HALF TO RICHARD FRANCHOT, OF NIAGARA FALLS, NEW YORK.

## PROCESS OF MAKING MOTOR FUEL.

No Drawing.

Application filed April 5, 1922. Serial No. 549,876.

To all whom it may concern:

Be it known that I, KARL P. McELROY, a citizen of the United States, residing at Washington, in the District of Columbia, have invented certain new and useful Improvements in Processes of Making Motor Fuel, of which the following is a specification.

This invention relates to a process of 10 making motor fuel; and it comprises a method wherein acetylene is passed through an acid solution, usually containing mercury, at a temperature of about 70° C. to convert a portion, but not all of it, into 15 acetaldehyde and the mixture of acetaldehyde vapor and acetylene, after drying is directly compressed into liquid form; all as more fully hereinafter set forth and as claimed.

20 Acetylene,  $C_2H_2$ , is one of the best known fuels for internal combustion engines but it is not used in practice because of the difficulty and danger of liquefaction and storage in tanks. Acetylene requires a pressure 25 of about 500 or 600 pounds, to keep it in the liquid form at ordinary atmospheric temperatures; and when so compressed in liquid form it is apt to explode. By passing acetylene through a solution containing sulfuric 30 acid or phosphoric acid of moderate strength and maintained at about 70° centigrade, some of the acetylene takes up water and becomes acetaldehyde; the  $C_2H_2$  reacting with  $H_2O$  to form  $C_2H_4O$ . The action is 35 much facilitated by the presence of mercury salts. The reaction is one well known for making acetaldehyde. It is, however, difficult to convert more than a portion of the acetylene in a single passage through the 40 liquid. In making acetaldehyde the mixture of excess acetylene and acetaldehyde coming from the acid liquid is scrubbed with water to recover the aldehyde, and the acetylene is returned for another treatment. 45 The acetaldehyde is recovered from the water solution by appropriate distillation. As its boiling point is very low (about 21° C.) condensation offers some difficulty. The acetaldehyde so recovered can be used 50 as a motor fuel but the expense of recovering it from the acetylene-acetaldehyde mix-

ture adds considerably to its cost; and moreover it is not nearly as good a fuel as the original acetylene; this being for the simple reason that it practically represents a hydrated acetylene. For the present purpose it may be regarded as a combination of acetylene and water.

I have found that if the usual method of making acetaldehyde be employed and in 60 lieu of attempting to recover the acetaldehyde, the effluent mixture of acetylene and acetaldehyde be directly cooled to dry it and then compressed, it is possible to make an excellent motor fuel with a cheap and 65 simple apparatus. A little acetaldehyde has a relatively enormous influence in facilitating the condensation of acetylene by pressure; and the liquefied acetylene containing acetaldehyde is not self-explosive. The 70 compressed liquid product being mainly acetylene is highly desirable as a motor fuel.

What I claim is:—

1. The process of making a motor fuel which comprises passing acetylene through 75 an acid solution in order to convert part but not all of it into acetaldehyde, drying the mixture of acetylene and acetaldehyde to remove water vapor and directly compressing into a liquid.

2. The process of making a motor fuel which comprises passing acetylene through an acid solution containing mercury in order to convert part but not all of it into acetaldehyde, drying the mixture of acetylene and acetaldehyde to remove water vapor and directly compressing into a liquid.

3. In methods of treating acetylene for the purpose of hydration to aldehyde by 90 passing such acetylene into intimate contact with acid liquids the process of making a useful combustible product which comprises collecting effluent gas and vapors leaving the hydrating apparatus, separating water from the mixture and compressing 95 the residual mixture into liquid form, unchanged acetylene present being aided in liquefaction by aldehyde present.

In testimony whereof, I have hereunto affixed my signature.

K. P. McELROY.